

Sept. 25, 1928.

1,685,640

J. M. LEAVER

# METHOD AND APPARATUS FOR MAKING ARTIFICIAL SILK

Filed Sept. 3, 1924



FIG. 1

BY

James M. Leaver.  
Julian A. Bried.  
his ATTORNEY.

## UNITED STATES PATENT OFFICE.

JAMES M. LEAVER, OF OAKLAND, CALIFORNIA, ASSIGNOR TO THE PACIFIC LUMBER COMPANY, OF SAN FRANCISCO, CALIFORNIA, A CORPORATION OF MAINE.

## METHOD AND APPARATUS FOR MAKING ARTIFICIAL SILK.

Application filed September 3, 1924. Serial No. 735,625.

This invention relates to the forming or so-called "spinning" of threads from viscous solutions generally, and particularly to the spinning of such threads in the making of 5 artificial silk.

The objects of my invention are to provide a method and apparatus for the above mentioned purpose which will be simpler and more effective than any with which I 10 am acquainted.

It might be mentioned that in the earlier methods of spinning artificial silk the filaments composing the threads were ejected from very minute orifices into various setting or precipitating baths, and gave much trouble through stoppage of the orifices due to their fineness; and that recently more attention has been directed to the use of larger orifices followed by stretching of the formed 20 thread or filament after precipitation, and to a certain extent during the forming thereof, and to a slight extent just prior to the setting of the filaments.

But I have found that if the nozzles are 25 considerably larger than heretofore used and the viscous solution is fed therethrough under a constant pressure; maintained either by pumping or gravity; and permitted to fall vertically from the nozzle 30 through a considerable air space (usually from one to several feet) that the method at once assumes a totally different commercial aspect, for the thread filaments, or rather the viscous streams from which they 35 are formed, in falling this relatively great distance take on the acceleration due to gravity which backed up by the feeding pressure of the material results in a very high speed of production, while at the same 40 time the great distance of falling through the air reduces the filaments to any desired fineness of perfect rotundity.

This however is not the end of my 45 process or method for great difficulty is found in properly setting such high speed minute streams into filaments in proper orderly arrangement or relation one to the other, and without breakage. The ordinary funnel and liquid methods are entirely too 50 violent in their mechanical action, for, unless the setting liquid has a surface speed of travel substantially synchronous with that

of the falling filament streams, yet without violent agitation, good results cannot be secured, and also, after the initial setting 55 it is desirable that the speed of flow of the solution and travel of the filaments should not be retarded, but should if possible always tend to increase somewhat until the 60 filaments are twisted or otherwise compacted into a thread and wound upon a receiving reel for washing and drying.

My apparatus for carrying out the above described method of producing threads from viscous material is shown in the accompanying drawings and in which Figure 1 is an elevation of my apparatus on a reduced scale 65 and with some of its parts shown in section, Figure 2 is a plan view of the ejecting nozzle shown approximately full size, Figure 3 is a cross section of the nozzle taken along the line 3—3 of Figure 2 showing the interior form of the device with a small feeding well above each orifice, Figure 4 is an enlarged representation of a portion of 70 my special variable pitch open helicoid filament compacting device, and Figure 5 is a front view of the precipitating chute which receives and guides the filaments to 75 thread formation and with ever increasing speed delivers them into the helicoid device.

In further detail the apparatus comprises a suitable frame 1 supporting a receptacle 2 for the viscous solution, and a receptacle 3 for the setting solution.

The viscous solution is maintained at a 80 constant level 4 within the receptacle or fed thereto under constant pressure by any suitable means not shown, and the setting liquid 5 is maintained in its receptacle in a similar manner, so that a perfectly uniform flow of either solution may be obtained.

From the bottom of the setting solution receptacle extends a pipe 6 controlled by a valve 7 for discharging the solution into a 85 well 8 supported just beneath the lower end 6' of the pipe, and from the well extends a downwardly inclined chute 9 connected to the well by a flat portion 10 for delivery of an even sheet of liquid to the chute from the surface 5' of the liquid in the well.

The chute has an increasing incline towards its lower end, terminating in a vertical drop, and a pair of sides 11 are pro-

vided which converge at the lower end of the chute as shown in Figure 5.

From the viscous solution receptacle extends a pipe 12 having a lower section 12' telescoping thereover and adjustable therewith by means of a clamp screw 13.

The lower section 12' has a control valve 14 and carries at its extreme lower end a multiple nozzle 15 for ejecting a plurality of viscous streams directly downward as shown at 16 to be intercepted by the flowing sheet of setting solution from the well, and which "sets" or precipitates them to the form of filaments and diverts them at an angle all to one side of the path of falling of the streams.

The distance from the nozzle to the point of impingement of the streams with the setting solution determines the fineness of the filaments, and this is also governed by the viscosity of the viscous solution employed and the size of the nozzle openings, but may be roughly stated to be about a foot or more when discharging a ten per cent solution of viscose from openings of about a millimeter or more depending somewhat on the force of the discharge of the material from the openings and the size of the filaments desired. With orifices an eighth of an inch in diameter and with a foot head of ten per cent solution above the nozzle, several feet of air space between the nozzle and setting bath produced very fine filaments at a very high speed of production.

Figure 2 shows in plan the full size arrangement of a nozzle successively employed, and discharging thirty streams through the orifices 17. The orifices are arranged in parallel rows and the nozzle is rotated with the telescopic pipe 12' to bring it to an angle with the travel of the setting solution in the chute so that the filaments will be carried to the left of the falling streams in side by side relation without interference, as shown in Figure 2 at 18 and as they are also designated in the chute 9 in their descent after first contact with the setting solution.

The nozzle may be constructed in the ordinary manner of small inserted tubes, but I show a simple way of forming it from a plate 19 grooved at 20 in opposite directions to form the discharging necks 21 through which the orifices 17 are drilled. Just above each orifice is a larger one 22 to serve as a feeding well for its particular orifice, and above the feeding wells the metal may be tapered to the wells by grooving as described for the face of the nozzle, or by countersinking, either construction being indicated at 23. The plate may be soldered to the tubular reservoir portion 15 along the dotted line 24 or made integral.

The filaments 18 it will be observed are in the form of a flat ribbon as they flow down the chute and the converging sides of the

chute gradually force the ribbon together to a thread like form, and with increasing speed of travel as they enter the helicoidal twister 25.

This device takes the form of a helicoidal chute, preferably of longer pitch at the upper end as indicated at 25' and progressively changing to a shorter pitch at the lower end as indicated at 25" so that the thread 18' enters gently and is spun around and compacted with increasing rapidity as it progresses, then gently ejected from the gradual curve 26 at the lower end as a compacted thread 18".

A portion of my helicoidal device is shown enlarged in Figure 4 and it will be seen that it is preferably an open chute having an outer wall 25<sup>a</sup>, and a lower wall or bottom 25<sup>b</sup>, and a central core 25<sup>c</sup>.

In passing through this device with great speed the solution tends to hug the outer wall and the thread is compacted around the core, therefore it is desirable that the gradual change of pitch of the chute should be such as to compensate for the acceleration due to gravity to maintain a substantially uniform progress of the thread through the device, so that it will not be stretched against the core and slowed up thereby; but fair results may be secured even with a chute of constant pitch if properly proportioned.

It should be noted that the helicoid chute, as well as the upper chute 9, being entirely open on top for their full length, it is simplicity itself to start the filaments therethrough in beginning work, and that any initial blocking up of the passages may be instantly removed as there is no complicated rifled or rotating closed tubular devices difficult of access in case of trouble, or in cleaning up, tho I wish to say that whatever novelty my helicoidal device possesses even if made with closed sides I wish to cover in my claims hereto appended.

From the helicoidal chute the compacted thread 18" descends with the setting solution to a tank 27 where the solution is maintained at a fixed level 5" by any suitable means not shown, and the thread is passed over a wheel 28 revolvable in the solution as indicated.

From the wheel 28 the thread passes through the solution to another wheel or reel 29 also revolving in the solution in the same direction but at a greater surface speed so as to stretch the thread at the point A between the wheels.

In commercial production the wheel or reel 29 upon which the thread is wound, may advantageously be given a reciprocatory motion in an axial direction by any of the well known means of so doing, so as to wind the thread in crossed layers upon its surface.

The wheel 28 may be a retarded idler, or a positively driven one as shown from the

wheel 29 through means of the chain indicated at 30, and the power to drive the winding wheel 29 delivered from any source of power through the chain indicated at 31 passing over a sprocket 31' secured either to the wheel or to its axle.

It is desirable that the final thread B be wound upon a detachable ring or band 32 slipped over the rim of the wheel 29 so that when sufficient thread is wound upon it the rim may be quickly slipped off for replacement with another, and to facilitate this procedure both wheels are revolvably supported on axles projecting from one side only with the other sides of the wheels free, thus making it a very simple matter to change rims or start the thread over the wheels in the beginning, or after placing a fresh rim in place.

Upon considering the apparatus as described it will be seen that no obstruction passes the path of the thread at any point of its making, so that it is freely accessible at any point from the discharge nozzle to the finished thread upon the reel 29, thus greatly facilitating starting the filaments through the apparatus, observing their proper operation at all points of the process, removing stoppage material in getting the apparatus properly adjusted, and in taking care of the finished product.

I claim:—

1. The method of forming thread filaments from viscous solutions, which consists in discharging the material downward in a plurality of streams, permitting the streams to fall through the air to reduce them in diameter to a fraction of their starting diameter, and receiving the falling streams on a moving sheet of setting solution having a surface speed substantially synchronous with that of the falling streams at their point of contact therewith.

2. The method of forming thread filaments from viscous solutions, which consists in discharging the material downward in a plurality of streams, permitting the streams to fall through the air to reduce them to a fraction of their starting diameter, and receiving them on a flat moving sheet of setting solution having a surface speed of travel substantially synchronous with the speed of the falling streams at their point of contact therewith.

3. The method of forming thread filaments from viscous solutions, which consists in discharging the material downward in a plurality of streams, permitting the streams to fall through the air to reduce them to a fraction of their starting diameter, and of receiving them on a moving sheet of setting solution having a speed substantially equal to that of the falling streams at their point of contact therewith and of progressively increasing speed thereafter.

4. The method of forming thread filaments from viscous solutions, which consists in discharging the material downward in a plurality of streams, permitting the streams to fall through the air to reduce them in diameter to a fraction of their starting size, and of receiving them on a moving sheet of setting solution traveling at a descending incline to carry the filaments all in a common angular direction from their points of contact with the solution in falling.

5. The method of forming thread filaments from viscous solutions, which consists in discharging the material downward in a plurality of streams, permitting the streams to fall through a space to reduce them to a fraction of their starting diameter, and of receiving them on a moving sheet of setting solution traveling across their path of falling, said streams being arranged to fall in a manner to be carried away with said moving sheet of setting solution substantially in the form of a flat ribbon.

6. The method of forming thread filaments from viscous solutions, which consists in discharging the material downward in a plurality of streams, permitting the streams to fall through a space to reduce them to a fraction of their starting diameter, and of receiving them on a moving sheet of setting solution traveling across their path of falling, said streams being arranged to fall in a manner to be carried away with said moving sheet of setting solution in the form of a flat ribbon with the filaments in side by side relation.

7. The method of forming thread filaments from viscous solutions, which consists in discharging the material downward in a plurality of streams, permitting the streams to fall through a space to reduce them to a fraction of their starting diameter, and of receiving them on a moving sheet of setting solution traveling at a descending incline across their paths of falling whereby they are carried away in the form of a flat ribbon, and of then concentrating the filaments into a thread.

8. The method of forming thread filaments from viscous solutions, which comprises discharging the material downward in a plurality of streams, permitting the streams to fall through a space sufficient to reduce them to a fraction of their starting diameter, receiving them on a moving sheet of setting solution traveling across their path of falling, converging the filaments thus formed to a thread-like form and of then passing them downwardly through a helicoidal path.

9. The method of forming thread filaments from viscous solutions, which comprises discharging the material downward in a plurality of streams, permitting the streams to fall through a space sufficient

to reduce them to a fraction of their starting diameter, receiving them in a moving bath of setting solution traveling across their path of falling, converging the filaments thus formed to a thread-like form and passing them together with the bath downwardly through a helicoidal path of progressively decreasing pitch.

10. The method of forming thread filaments from viscous solutions, which comprises discharging the material downward in a plurality of streams, permitting the streams to fall through a space to reduce them to a fraction of their starting diameter, 15 receiving them in a bath of setting solution moving across their path of falling, converging the filaments thus formed to a thread-like form and passing the converged filaments and bath downwardly through a 20 helicoidal path at a substantially uniform speed of travel while passing therethrough.

11. The method of forming thread filaments from a viscous solution, which comprises discharging the solution downward in 25 a plurality of streams, permitting the streams to fall through space to reduce them to a fraction of their starting diameter, receiving them in a bath of setting solution moving across their path of falling, converging the filaments thus formed into a thread-like form and passing them together with the bath downwardly through a helicoidal path of progressively decreasing pitch while maintaining the speed of travel 30 through said path substantially constant.

12. The method of forming thread filaments from a viscous solution, which comprises discharging the material downward in a plurality of streams, permitting the 40 streams to fall through a space to reduce them to a fraction of their starting diameter, receiving them in a traveling bath of setting solution passing across their path of falling, converging the filaments thus 45 formed into a thread-like form and then passing them together with the setting solution through a helicoidal path and into a further bath of the setting solution and of therein mechanically stretching the 50 thread.

13. The method of forming thread from a viscous solution, which consists in discharging the material downward in a plurality of streams, permitting the streams to fall 55 through a space to reduce them to a fraction of their starting diameter, receiving them on a moving sheet of setting solution traveling across their paths of falling whereby they are carried to one side of their place of falling, compacting the filaments thus formed into a thread, and of stretching the thread after compacting all while traveling and immersed in the setting solution.

14. In a method of forming thread as 60 specified in claim 13, the compacting of the

filaments being carried out substantially without tensioning the same.

15. The method of stretch spinning of thread filaments from viscose solution, which comprises discharging a stream of cellulose sodium xanthate solution downward through an air space before setting, and intercepting the stream in a setting solution at a vertical distance under the point of discharge sufficient to reduce the unset stream of viscose 75 to a fraction of its starting diameter so as to form a precipitated filament of reduced diameter.

16. The method of stretch spinning of thread filaments from viscose solution, 80 which comprises discharging a stream of cellulose sodium xanthate solution downward through an air space before setting, and intercepting the unset stream in a setting solution at a vertical distance under 85 the point of discharge of the stream not less than one hundred times the diameter of the stream at its point of discharge.

17. For the forming of thread filaments from a viscose solution, an inclined chute, 90 means for maintaining a stream of viscose setting bath running down said chute, a multiple stream viscose ejector spacedly arranged above said chute and bath directed to discharge streams of viscose downwardly 95 through an air space to the bath in the inclined portion of the chute for travel with said bath.

18. In apparatus as specified in claim 17, 100 said chute having converging sides adapted to force the filaments together into a thread-like form as they pass along the chute.

19. For the formation of thread filaments from viscous solutions, means for discharging streams of the solution into a setting 105 solution, means for guiding the filaments while in the solution into thread relation, and a downwardly directed helicoidal chute arranged to receive the filaments so related together with the setting solution and 110 adapted to compact the filaments into a thread in descent therethrough.

20. In a structure as specified in claim 19, 115 said chute being open substantially for its length whereby the thread is accessible therealong.

21. In a structure as specified in claim 19, 120 said chute being of decreasing pitch in its downward descent.

22. For the formation of thread filaments from a viscous solution discharged from an ejector and set in a precipitating solution, a device into which the filaments are guided comprising a helicoidal channel directed 125 downwardly and arranged to receive the filaments and setting solution at its upper end.

23. In a structure as specified in claim 22, said helicoidal channel having a progressively varying pitch.

24. In a structure as specified in claim 130

- 22, said helicoidal channel having a central rod around which the filaments travel in their descent.
25. In a structure as specified in claim 5 22, said helicoidal channel being open on top from end to end.
26. Apparatus for forming a band of artificial silk filaments comprising a spinning nozzle provided with a plurality of 10 rows of ejection orifices directed downwardly, means for removing a bundle of falling filament streams from said nozzle in a lateral direction from the path of falling, and means for varying the angle of the 15 lateral removal of the streams with respect to the rows of orifices, whereby to produce a band of evenly spaced filaments spaced a distance apart depending on the relative angle of removal with respect to the rows 20 of orifices.
27. For the forming of thread filaments from viscose solution, an inclined open chute, means for maintaining a viscose setting bath running down said chute, a 25 multiple stream viscose ejector spacedly positioned above said chute and bath directed to discharge streams of viscose downwardly through an air space to the bath in the inclined portion of the chute, and means 30 for varying the separation of the ejector and the solution in the inclined chute.
28. In an apparatus as specified in claim 17, said chute having an increasing incline at its discharge end discharging both bath 35 and filaments therefrom in a common downward direction.
29. For the formation of thread filaments from a viscose solution, means for ejecting the solution in a plurality of streams into a setting solution, means for compacting the 40 filaments thus formed while in the solution to form a thread, means supporting the thread in the solution after compacting, and further means for stretching the thread after leaving said supporting means and 45 while still immersed in the solution.
30. In a structure as specified in claim 29, said further means comprising a device immersed in the solution over which the thread is guided, and a reel immersed in the solution 50 receiving the thread and rotated at a speed to cause stretching of the thread between the device and the reel.
31. In a structure as specified in claim 29, said further means comprising a roller 55 immersed in the setting solution and over which the thread passes, and a receiving reel for the thread, the roll and reel having different surface speeds for stretching the thread extending between them. 60
32. For the formation of a thread from a viscous solution, a multiple stream ejector for discharging the solution in a plurality of streams, means including a moving setting solution adapted to receive and set the 65 streams to fine filaments and for carrying same away from the point of contact of the streams therewith, means for compacting the filaments while being carried in the solution, and means for receiving the thread 70 thus formed, all of said means presenting a freely open side substantially the length of travel of the filaments and thread.

JAMES M. LEAVER.